

## UNITED STATES PATENT OFFICE

1,982,718

## ANTICARBURIZING COMPOUND

Walter G. Wittman, Indianapolis, Ind., assignor  
of ten per cent to Roger F. Marshall, Indian-  
apolis, Ind.

No Drawing. Application October 18, 1933,  
Serial No. 694,115

11 Claims. (Cl. 148—4)

This invention relates to an anticarburizing compound which is used in the case hardening of steel products to localize the carburizing effect. More particularly, the invention relates to a compound to be applied to such portions of the surface of the product as are not to be hardened and which prevents the carburizing of such portions.

In the case hardening process, the product to be hardened is packed in a carburizing compound and then heated to a desired temperature, at which temperature the carbon from the compound enters the pores of the product and, combining with the iron therein, makes the surface sufficiently high in carbon content to react to a further heat treating process for hardening. In many products, it is desirable that only a portion of the surface be hardened. In order to prevent the hardening of undesired parts of the surface, it has heretofore been the practice to coat such parts with an electrolytic plating of copper or other non-ferrous metal which mechanically prevents the carbon from penetrating the surface. This method is relatively expensive, requires considerable apparatus and also leaves an undesirable metallic coating on the product.

It has also been the practice to apply other coatings, such as ground fire clay or asbestos, which mechanically prevent the access of carbon to the parts which are not to be hardened. This method is difficult of use where the products require relatively rough handling in the packing operation since it is difficult to give the coating sufficient mechanical strength to resist such handling. Such coatings also require considerable time for drying before the product may be carburized. In certain cases, the drying time is three hours or more.

In the present invention, these objections are overcome by a coating compound which apparently performs its function chemically rather than mechanically, which leaves no visible residue upon the unhardened surface when the carburizing process is completed and which requires practically no drying time.

The compound forming the present invention in its most preferred form consists in a water solution of a salt or salts of copper or a similar metal and oxalic acid or a similar organic acid in which there is suspended an oxide of lead. For best results, I prefer to prepare the compound

with the ingredients in the following proportions, although these proportions may be varied within a considerable range:

|                 | Parts |
|-----------------|-------|
| Cupric sulphate | 5 1/2 |
| Cupric chloride | 2     |
| Oxalic acid     | 3     |
| Water           | 5     |
| Lead oxide      | 1     |
|                 | 60    |

The proportion of ingredients given are parts by volume and refer to a crushed crystalline form for the copper salts and the oxalic acid. The water is preferably distilled water and the lead oxide is preferably the monoxide, litharge, PbO, in powdered form.

In the use of the compound, the solution is applied to the parts to be protected from hardening either by dipping or by the use of a brush. The solution dries almost immediately, leaving the chemical ingredients of the compound in the form of a relatively thin coating precipitated on the surface of the product. The coating adheres so strongly to the surface that it can not be removed by ordinary rubbing but requires abrasion on an emery wheel or similar tool for removal. Contrary to the case with the mechanical coatings of the prior art, no amount of rough handling can remove the coating. The coated product is packed in the carburizing compound in the well known manner and heated as in the prior art. When removed from its packing, no trace of the anti-carburizing compound is visible, although it is possible that a certain amount of metallic copper or lead, or both, is deposited in the pores of the iron. The parts protected by the compound are not carburized and when heated treated, are found to be substantially as soft as when originally formed, while the unprotected parts are thoroughly case hardened.

The exact nature of the probable chemical reactions between the ingredients of the compound, the carbon or carbon monoxide of the carburizing compound and the iron is not known and no explanation thereof is attempted herein.

Where a thicker coating than usual is required, I add to the compound one part of powdered alum. This apparently acts as a coagulator to produce the desired thickness of coating and is useful for

carburizing operations longer than the ordinary.

The invention claimed is:

1. An anti-carburizing compound containing cupric chloride, oxalic acid, and a lead oxide.
- 5 2. An anti-carburizing compound containing cupric sulphate, cupric chloride, oxalic acid, and a lead oxide.
- 5 3. An anti-carburizing compound containing cupric chloride, a lead oxide, and an organic acid.
- 10 4. An anti-carburizing compound containing cupric chloride, cupric sulphate, a lead oxide, and an organic acid.
- 15 5. An anti-carburizing compound containing cupric chloride, cupric sulphate, oxalic acid, and litharge.
6. An anti-carburizing compound containing the following ingredients in substantially the proportions named:

|                    | Parts |
|--------------------|-------|
| 20 Cupric sulphate | 5 1/2 |
| Cupric chloride    | 2     |
| Oxalic acid        | 3     |
| Water              | 5     |
| Lead oxide         | 1     |
|                    | 1     |

25

| Parts |    |
|-------|----|
| 5 1/2 | 80 |
| 2     |    |
| 3     |    |
| 5     |    |
| 1     |    |
| 1     | 85 |

7. An anti-carburizing compound containing the following ingredients in substantially the proportions named:

| Parts           |       |
|-----------------|-------|
| Cupric sulphate | 5 1/2 |
| Cupric chloride | 2     |
| Oxalic acid     | 3     |
| Water           | 5     |
| Lead oxide      | 1     |
| Powdered alum   | 1     |

8. An anti-carburizing compound containing cupric chloride, an organic acid a lead oxide, and a coagulator.

9. An anti-carburizing compound containing cupric chloride, cupric sulphate, an organic acid, a lead oxide, and a coagulator.

10. An anti-carburizing compound containing cupric chloride, oxalic acid, a lead oxide, and a coagulator.

11. An anti-carburizing compound containing cupric chloride, cupric sulphate, oxalic acid, a lead oxide, and a coagulator.

WALTER G. WITTMAN.

100

30

105

35

110

40

115

45

120

50

125

55

130

60

135

65

140

70

145

75

150